

Nov. 20, 1951

L. W. RAINARD

2,575,839

## PROCESS FOR CRIMPING UNCROSSLINKED FIBERS

Filed Dec. 15, 1948

Fig. 2



INVENTOR.  
LEO W. RAINARD

BY

W. G. F.

**ATTORNEY**

## UNITED STATES PATENT OFFICE

2,575,839

## PROCESS FOR CRIMPING UNCROSS-LINKED FIBERS

Leo W. Rainard, Nyack, N. Y., assignor to Alexander Smith, Incorporated, a corporation of New York

Application December 15, 1948, Serial No. 65,440

5 Claims. (Cl. 19—66)

1

This invention relates to the treatment of uncross-linked fibers, and more particularly to a process for imparting an artificial crimp to vegetable fibers and uncross-linked synthetic thermoplastic fibers, and has for an object to provide a fiber of the above type having novel and improved characteristics.

Another object is to produce a fiber of the above type characterized by a predominance of sharp, angular bends or crimps with the portions between bends substantially straight.

Another object is to provide an artificially crimped fiber of the above type having improved carding and spinning characteristics.

Other objects and advantages will be apparent as the nature of the invention is more fully disclosed.

In accordance with one embodiment of this invention, the crimp is produced mechanically by feeding the fibers in the form of a roving or slubbing between feed rolls into a crimping chamber which is maintained full of fibers under a predetermined temperature and back pressure. As the fibers are forced into the crimping chamber, they are laid in a zig-zag form and are pressed to form angular bends or crimps with intervening straight portions, the length of which depends upon several factors, such as the nature of the fibers and the temperature and pressure to which the fibers are subjected in the crimping chamber. The temperature in the crimping chamber should be in the range below which the natural resilience of the fibers resists deformation and above which degradation occurs, the relationship being such that the fibers are brought to the plastic condition necessary for the formation of a permanent crimp. The crimp is set by rapid cooling in a cooling chamber.

The novel features which are characteristic of this invention will be better understood by referring to the following description, taken in connection with the accompanying drawings in which a specific form of crimping apparatus has been set forth for purposes of illustration.

In the drawings:

Fig. 1 is a side elevation of an apparatus embodying the present invention;

Fig. 2 is a top plan view thereof on a larger scale; and

Fig. 3 is a vertical section taken along the line 3—3 of Fig. 2.

Referring to the drawings more in detail, the crimpler is shown as comprising a frame 10 carrying a pair of feed rolls 11 and 12 and drive shaft 13. The shaft 13 is journalled in the frame 10 and carries a pinion 15 and a sprocket 14 which is driven by suitable means, not shown. The feed roll 11 is keyed to a shaft 16 journalled in bearing blocks 17 fixed to the frame 10 and carrying a gear 18 meshing with the pinion 15.

2

The feed roll 12 is keyed to a shaft 20 journalled in bearing blocks 21 which are slidable in the frame 10. The roll 12 is held in pressure engagement with the material fed between the rolls by springs 22 seated around threaded rods 23 which bear against the bearing blocks 21. The rods 23 extend through a bracket 24 attached to the frame 10 and carry nuts 25 and adjusting knobs 26. The nuts 25 are held against rotation by the frame 10. The springs 22 are seated between the nuts 25 and the bracket 24 and their tension may be adjusted by means of the knobs 26.

The shaft 20 carries a gear 30 meshing with the gear 18. The gears 18 and 30 have teeth of sufficient depth to remain in mesh throughout the normal range of sliding movement of the shaft 20 during the operation of the crimpler.

Positioned below the rolls 11 and 12 is a vertical tube 33 having a conical bore 34, forming a cooling chamber. The tube 33 is attached to a saddle 35 having a tapered central bore 36 forming a crimping chamber and having a curved upper surface 37 conforming to the bight of the rolls 11 and 12 and machined to have a slight running clearance from the surface of the rolls. The saddle 35 is attached to the frame 10 by suitable means and is formed with a plurality of radial passages 42 for the injection of a heating agent such as hot air into the crimping chamber. The radial passages 42 communicate with an annular passage 43 in the saddle 35 which is closed by a collar 44 to form an inlet manifold. The fluid is supplied to the annular passage 43 by a pipe 45 registering with a port 46 in said collar.

35 A cooling agent, such as cold air, is introduced into the cooling chamber through radial passages 47 communicating with an annular passage 48 in the tube 33 which is closed by a collar 49. A cold air supply duct 57 communicates through 40 the collar 49 with the annular passage 48. The passages 47 are preferably located about midway of the length of the cooling chamber so that the entire mass of fibers therein will be subjected to the cooling air.

45 At its lower end the tube 33 carries a flanged extension 50 to which a pair of doors 52 are hinged by hinges 53 and are held closed against the tapered end 54 of the extension 50 by weights 55 attached to arms 56 secured to the doors.

In the operation of the crimpler, the rolls 11 and 12 are driven by any suitable source of power and the fibers to be crimped are fed thereto over a guide roll 58, preferably in the form of a rope or a web 59. The fibers are held in the crimping and cooling chambers by the doors 52 until they have been packed sufficiently to force the doors slightly open against the force of the weights 55. The back pressure of the packed fibers causes the fibers which are being forced against the packed fibers by the feed rolls to be folded over in zig-zag

crimps, the spacing of which depends upon the nature of the fibers, the temperature, and the back pressure.

The heating agent, such as hot air, is introduced through the pipe 45 and passages 42 into the mass of packed fibers and is controlled so as to raise the fibers in the crimping chamber to the desired temperature for crimping.

The raw fibers may be treated in the usual manner to form stock. This pretreated stock is fed directly at a uniform rate to the feed rolls 11 and 12 of the crimper or may be fed to a web-forming device, such as a card, and fed as a web or condensed into a rope which is fed to the feed rolls 11 and 12 as a sliver or slubbing 59. If a more uniform feed is required, the stock may be picked and carded and condensed to a rope for the above purpose after one or more stages of carding. A uniformity in density of feed stock is preferred to prevent jamming or slipping at the feed rolls or undue lateral movement of the feed rolls.

In either case, the fibers are stuffed by the feed rolls 11 and 12 into the crimping chamber and through the cooling chamber and are forced out of the bottom of the cooling chamber against the pressure exerted by the discharge doors 52.

The back pressure at the entrance of the crimping chamber controls the size of the crimp, a higher pressure causing a finer crimp (more crimps per inch) and vice versa.

For higher temperatures, steam under pressure may be used. The quality of steam should be selected to cause the fibers to reach the desired temperature and moisture content. Due to the packing of the mass of fibers, they are relatively impermeable to steam and steam pressures suited to produce the desired high temperatures may be used.

The hot fluid may be injected under conditions to raise the temperature of the fibers to a point to bring the fibers to a plastic condition to permit the crimps to form therein, for example, to a temperature of 212° F. to 300° F. and the cooling in the cooling zone may be controlled to cool the fibers to a temperature below that at which they are in a plastic condition so as to set the crimps while the fibers are still held under pressure and before discharge thereof from the cooling zone. The time should be sufficient to permit all of the fibers to reach the necessary temperatures in the crimping and cooling zone, one or two minutes usually being sufficient.

The crimped fibers emerge from the crimper in the form of a very condensed tow or rope, which is easily opened and separated.

The fibers may be carded, formed into a roving and spun in the usual manner and skein dyed if desired, or they may be picked to open the fibers and stock dyed after which they may be carded and spun into yarn. The entanglement of the fibers due to the predominance of angular bends causes the fibers to interact more strongly and in carding the uniform distribution of the fibers over the card cylinder is greatly facilitated. The sliver from the card cylinder is more readily condensed into a uniform round and full roving which can be drawn out to produce a substantial reduction in diameter and spun without breaking. The yarn made from such artificially crimped fibers is characterized by more resilience and fullness than similarly prepared yarn made from fibers which have not been subjected to this process of crimping. The artificially crimped

fibers may also be blended with other fibers and formed into yarn if desired.

This process is particularly applicable to vegetable fibers, such as cotton, hemp, jute, ramie and flax, and to uncrosslinked thermoplastic synthetic fibers, such as viscose rayon, acetate rayon, nylon, condensation products of terephthalic acid and glycol (terylene) and polyvinylidene chloride products, either in staple or filament form. These fibers have the characteristic of being thermoplastic to an extent such that they may be softened by heat to permit mechanical crimping and set immediately on cooling.

The process and apparatus may be varied as will be apparent to a person skilled in the art.

What is claimed is:

1. The method of imparting a permanent artificial crimp to vegetable fibers and uncrosslinked thermoplastic synthetic fibers, which comprises gripping said fibers between closely spaced conveyor surfaces discharging into a substantially closed crimping zone, and forcing the gripped fibers into said zone against the pressure of a mass of fibers held compacted under pressure in said zone, said pressure being adapted to cause the fibers to be progressively folded over and crimped as they are delivered from said conveyor surfaces, holding the mass of crimped fibers compacted under a substantially constant pressure to retain the crimp therein, injecting a hot fluid into the mass of fibers in said zone to heat the fibers to a temperature to bring the fibers to a plastic condition in which permanent angular bends are formed at the folds therein, advancing said fibers while held under said pressure through a cooling zone, cooling the fibers in said cooling zone to a temperature below that at which they are in a plastic condition to set said crimps and discharging the crimped fibers from said cooling zone.

2. The method set forth in claim 1 in which a cooling fluid is introduced into the mass of fibers in said cooling zone.

3. The method set forth in claim 1 in which hot air is introduced into the mass of fibers in said crimping zone for heating the same.

4. The method set forth in claim 1 in which hot air is introduced into the mass of fibers in said crimping zone for heating the same, and cold air is introduced into the mass of fibers in said cooling zone.

5. The method set forth in claim 1 in which the fibers are heated to from 212° F. to 300° F. in the crimping zone and are cooled below 180° F. in the cooling zone.

LEO W. RAINARD.

#### REFERENCES CITED

The following references are of record in the file of this patent:

#### UNITED STATES PATENTS

| Number    | Name             | Date           |
|-----------|------------------|----------------|
| 2,139,543 | Finlayson et al. | Dec. 6, 1938   |
| 2,204,341 | Cobb             | June 11, 1940  |
| 2,208,632 | Dreyfus          | July 23, 1940  |
| 2,300,791 | Lodge            | Nov. 3, 1942   |
| 2,311,174 | Hitt             | Feb. 16, 1943  |
| 2,321,757 | Lodge            | June 15, 1943  |
| 2,394,165 | Getaz            | Feb. 5, 1946   |
| 2,428,046 | Sisson et al.    | Sept. 30, 1947 |
| 2,434,533 | Wurzburger       | Jan. 13, 1948  |
| 2,504,183 | Croft            | Apr. 18, 1950  |
| 2,505,618 | Hammerle         | Apr. 25, 1950  |
| 2,514,557 | Pfau             | June 11, 1950  |